

# UNITED STATES PATENT OFFICE.

CHARLES MUSIOL, OF BRUSSELS, BELGIUM.

## ENAMEL FOR ENAMELING ARTICLES IN SHEET METAL OR CAST METAL.

1,332,058.

Specification of Letters Patent. Patented Feb. 24, 1920.

No Drawing.

Application filed June 12, 1919. Serial No. 303,796.

To all whom it may concern:

Be it known that I, CHARLES MUSIOL, engineer, 16 Rue de la Bigorne, Brussels, Belgium, have invented certain new and useful Improvements in Enamel for Enameling Articles in Sheet Metal or Cast Metal; and I do hereby declare the following to be a full, clear, and exact description of the invention, such as will enable others skilled

10 in the art to which it appertains to make and use the same.

The foundation coatings heretofore in use, as well as shining or bright and colored glazings used for enameling articles of sheet 15 metal or cast metal are composed of mixtures of silicates, fluorates and borates, to which are added coloring materials such as metallic oxids. Borax or compounds of boron are always necessary when producing 20 enamels from the hereinbefore mentioned ingredients. The enamels obtained in this manufacture always include boron. By the addition of boric acid the enamels fuse easily and adapt themselves to the eventual 25 expansions of the enameled metals, but these results are obtained by the sacrifice of duration of the enamels.

Heretofore, enamels were at disposal other than borosilicated glasses, which are 30 easily fusible. The glazings comprising lead are the only exceptions, but owing to the poisonous quality of the lead, they are unsuited for several uses, for instance kitchen utensils.

The net cost of all enamels in practical 35 use is regulated by the quantity and the price of the compounds of boron therein contained, and the result of this is that thirty-five to fifty-five per cent. and even seventy-five per cent. of the total value of 40 the fused enamels are represented by the quantity of borax used.

According to the present invention it is possible to provide valuable enamels which are independent of the compounds of boron, 45 such compounds not being used in the manufacture of these enamels. For the production of these enamels without boron, the following are used: feldspar, fluorid of sodium, fluorid of aluminum, fluorspar, calcareous spar, silico-fluorid of sodium, kaolin or chine-clay, cryolite, magnesia, potash, quartz, sand, saltpeter, soda, alumina, as well as the known opacifiers, metallic oxids 50 and coloring matters. In the manufacture 55 of these enamels no use is made of milk-glass or opal glass, nor of products containing lead or arsenic, nor of compounds of boron. The quantities of the various materials in the mixing for the manufacture of 60 these enamels without boron are chosen according to the required qualities of the enameled articles; fusibility, resistance, hardness, stability, resistance to acids, opacity, 65 color, etc.

For a whole series of enamels use is made 65 of combinations of substances which are mixed as indicated in the following list:

### Rough mixture.

|                                                                    | Chemicals.                                                                                | White. |     | Enamel, bright. |     | Colored. |     |
|--------------------------------------------------------------------|-------------------------------------------------------------------------------------------|--------|-----|-----------------|-----|----------|-----|
|                                                                    |                                                                                           | From   | To  | From            | To  | From     | To  |
| Silicate (triple) of alumina, soda and lime, mixed with fluorids.  | Saltpeter.....                                                                            | 1.0    | 6.5 | 1.0             | 6.5 | 1.0      | 6.5 |
|                                                                    | Soda.....                                                                                 | 15     | 28  | 15              | 28  | 15       | 28  |
|                                                                    | Quartz, sand, or flint.....                                                               | 15     | 35  | 15              | 35  | 15       | 35  |
|                                                                    | Feldspar.....                                                                             | 18     | 40  | 18              | 40  | 18       | 40  |
|                                                                    | Kaolin or clay.....                                                                       | 0      | 8   | 0               | 3   | 0        | 5   |
|                                                                    | Fluorspar.....                                                                            | 1.5    | 15  | 1.5             | 15  | 1.5      | 15  |
|                                                                    | Silico-fluorid of sodium.....                                                             | 0      | 15  | 0               | 0   | 0        | 15  |
|                                                                    | Cryolite.....                                                                             | 0      | 15  | 0               | 0   | 0        | 15  |
|                                                                    | Chiolite.....                                                                             | 0      | 15  | 0               | 0   | 0        | 15  |
|                                                                    | Oxid of antimony.....                                                                     | 0      | 6   | 0               | 1   | 0        | 5   |
|                                                                    | Leuconine.....                                                                            | 0      | 10  | 0               | 0   | 0        | 0   |
|                                                                    | Magnesia.....                                                                             | 0      | 2   | 0               | 1   | 0        | 1   |
|                                                                    | Coloring-oxid such as: oxid of cobalt, oxid of nickel, oxid of manganese, oxid of chrome. | 0      | 0   | 0               | 0   | 0        | 8   |
| Mill addition in percentage of the weight of melted rough mixture. | Clay.....                                                                                 | 4      | 8   | 4               | 8   | 4        | 8   |
|                                                                    | White coloring products such as: oxid of tin, substitutes for oxid of tin, etc.           | 0      | 10  | 0               | 0   | 0        | 0   |
|                                                                    | Coloring matters.....                                                                     | 0      | 0   | 0               | 0   | 0        | 20  |
|                                                                    | Magnesia.....                                                                             | 0      | 0.5 | 0               | 0.5 | 0        | 0.5 |

The basis or support of the new enamel and lime, fusing easily, mixed with fluorids. 70 without boron is an aluminum silicate, soda. Owing to the fact that the raw materials

frequently differ to some extent according to their origin the composition of the final product is of great consequence for obtaining the enamel desired. The theoretical 5 composition of the enamel, after it has been fused in the fire, consequently without taking into consideration the loss of fluorid, must be maintained within the percentage limits given hereinafter, for obtaining use-  
10 ful enamels:

| Elements.                      | From—       |
|--------------------------------|-------------|
| Na <sub>2</sub> O              | 10 % to 20% |
| K <sub>2</sub> O               | 1. 5% " 5%  |
| CaO                            | 1. 5% " 6%  |
| 15 MgO                         | 0 % " 1%    |
| Al <sub>2</sub> O <sub>3</sub> | 5 % " 10%   |
| SiO <sub>2</sub>               | 50 % " 65%  |
| Fl                             | 1. 5% " 10% |
| Sb <sub>2</sub> O <sub>5</sub> | 0 % " 7%    |
| 20 SnO <sub>2</sub>            | 0 % " 9%    |

The white color is obtained, as heretofore, by means of known white coloring-materials and the various colorations are obtained by 25 means of metallic oxides and known coloring-matters.

The materials that are necessary for the mixing are weighed carefully, according to the quantities that have been found suitable 30 for the various sorts of enamels, mixed by hand or mechanically and melted together in the melting furnace. The melted mixture is then poured into water and ground in wet state together with the mill addition, previously carefully weighed. The enamels thus obtained are further mixed, if necessary, with carbonate of ammonia, after 35

which they are ready for the application on the articles to be enameled. The heating of the articles is effected according to their 40 purpose, thickness of walls, composition, etc., at a temperature from 800° to 1050° C., usually at a temperature of about 900° C.

The finished enamel according to the invention has a splendid luster, resists very 45 well high temperature, possesses a great tensile strength and considerable elasticity, and surpasses enamels containing boron by its resistance to the action of liquids and of acids of fruits, etc.

50 What I claim is:

1. An enamel without boron for enameling articles of sheet metal or cast metal, the basis or support of which is a triple silicate of aluminium, sodium and calcium, mixed 55 with fluorids.

2. An enamel without boron for enameling articles of sheet metal or cast metal, the basis or support of which is a triple silicate of aluminium, sodium and calcium, mixed 60 with fluorids and opacified.

3. An enamel without boron for enameling articles of sheet metal or cast metal, the basis or support of which is a triple silicate of aluminium, sodium and calcium mixed 65 with fluorids and colored by means of coloring materials.

In testimony whereof I affix my signature in presence of two witnesses.

CHARLES MUSIOL.

Witnesses:

EUGÈNE DEYON,  
CHARLES MERCHIE.